

Patented Sept. 19, 1950

2,522,802

# UNITED STATES PATENT OFFICE

2,522,802

## PRODUCTION OF YELLOW DYE IMAGES BY COLOR DEVELOPMENT

Donald E. Sargent and Robert C. Gunther,  
Easton, Pa., assignors to General Aniline &  
Film Corporation, New York, N. Y., a corpora-  
tion of Delaware

No Drawing. Application December 22, 1948,  
Serial No. 66,825

8 Claims. (Cl. 95—88)

1

The present invention relates to the preparation of yellow dye images by photographic color forming development.

One of the classic methods for the production of dyestuff images in photographic elements involves the incorporation in a monopack of non-diffusing color formers, the exposure of the monopack and the development therein of the desired subtractive color images by color development with a primary aromatic amino developer of the p-phenylenediamine type. The greatest virtue of this process resides in its simplicity, to wit, the production in one color development step of the three subtractive color images. One of the disadvantages of the process involves the nature of the dyes produced which are either of the azomethine or quinonimine type, and which are therefore quite fugitive in the presence of acid vapors, particularly of sulfur dioxide.

Schmidt and Tulagin, in their application Serial No. 640,382, now Patent No. 2,486,440, November 1, 1949, describe the production of azine dye images by the color development of an exposed silver halide emulsion with a 2,4-diaminoaniline in the presence of a color former which is preferably an aromatic compound containing at least one hydroxyl group linked to the aromatic structure. This process has as its greatest merit the fact that it yields dyestuff images which are much more stable, particularly to acid vapors, than are the azomethines or quinonimines.

However, such process as developed to the present time did not lend itself to the processing of multilayer film with the same simplicity as the older method, primarily because of the inability of operators to effectively produce a permanent yellow dye image simultaneously with magenta and cyan dye images upon color development. As stated the color formers generally employed in the azine method were of the phenolic type, and these invariably led to the formation of azine dyes which were cyan, blue, magenta, red or reddish-orange in color.

Attempts had been made to produce the yellow images by the employment as color formers of keto methylene compounds, such as acetoacetanilide, and the like. Such attempts were unsuccessful, however, since the images which were produced did not persist in the yellow form.

2

Such lack of success in synthesizing the yellow dye images by color development materially operated, against the adoption of this process for practical use despite the excellence of the dyes produced, for the reason that its adoption would require a step separate from that of color forming development of the cyan and magenta images to insure the formation of a permanent yellow image.

We have now discovered, very surprisingly indeed, that a permanent yellow dye image can be produced simultaneously with the cyan and magenta azine dye images by color forming development with a 2,4-diamino aniline in the presence of a keto methylene compound providing that the pH of the photographic element subjected to processing be adjusted with an alkali in a final phase of the processing operations until a yellow image clearly manifests itself.

It is an object of the present invention to color develop a developable silver halide emulsion with a 2,4-diaminoaniline in the presence of a keto methylene compound to produce a yellow dye image.

It is a further object of the present invention to color-develop a developable silver halide emulsion with a 2,4-diamino aniline in the presence of a keto methylene compound while adjusting the pH by means of an alkali in a final phase of the processing operation until a yellow image manifests itself.

Other and further objects of the invention will become apparent as the description proceeds.

The color forming developers which we employ, and which as stated are of the 2,4-diaminoaniline type, may be represented by the following structural formula:



wherein R is hydrogen or alkyl, i.e., methyl, ethyl, propyl, butyl, amyl or the like, and R<sub>1</sub> is an aliphatic radical such as alkyl as above, carboxy alkyl such as carboxy methyl, carboxy ethyl and the like, hydroxy alkyl such as hydroxy ethyl,

hydroxy propyl and the like, sulfo alkyl such as sulfomethyl, sulfopropyl, sulfobutyl and the like, or an aromatic radical such as aryl, i. e., phenyl, naphthyl and the like, carboxy aryl, i. e., carboxy phenyl, carboxy naphthyl and the like, sulfo aryl, i. e., sulfophenyl, sulfonaphthyl and the like, alkoxy aryl such as methoxy phenyl, methoxy naphthyl, ethoxy phenyl, butyroxy phenyl and the like, alkyl aryl such as toluyl, ethylphenyl, propylphenyl and the like, carboxy alkylaryl, such as carboxy methyl phenyl, carboxy ethyl phenyl and the like, carboxy alkoxy aryl, such as carboxy methoxy phenyl, carboxy ethoxy phenyl, hydroxy alkyl aryl such as hydroxy methyl phenyl, hydroxy ethyl phenyl and the like, and hydroxy alkoxy aryl such as hydroxy methoxy phenyl, hydroxy ethoxy phenyl and the like, R<sub>2</sub> is an aromatic or aliphatic radical as illustrated above, and X and Y are hydrogen, alkyl as above, sulfo, or carboxy. Preferably the compounds which are utilized are the N-substituted-4,6-diaminometanilic acids, in which case Y is hydrogen, and X is sulfo. It will be observed that in these compounds a carbon atom of the substituent groups represented by R and R<sub>2</sub> is directly linked to an amino nitrogen atom.

Such developers are described in the aforementioned Schmidt and Tulagin application, Serial No. 640,382, filed January 10, 1946. The developers may be used alone or in admixture.

Examples of suitable color forming developers are:

1. 2,4-di-(phenylamino)-aniline.



2. 6-(N-sulfomethyl-N-phenyl)-amino-4-phenylamino-metanilic acid.



3. 2,4-bis(3'-carboxyphenylamino)-aniline.



4. 4,6-bis-(phenylamino)-metanilic acid.



5. 4,6-bis-(4'-methoxyphenylamino)-metanilic acid.



6. 4-(2'-methoxyphenylamino)-6-(4'-methoxyphenylamino)-metanilic acid.



7. 4-(4'-methoxypyhenylamino)-6-(phenylamino)-metanilic acid.



8. 4,6-bis(2'-methoxyphenylamino)-metanilic acid.



9. 4-(3'-carboxyphenylamino)-6-(4'-methoxyphenylamino)-metanilic acid.



10. 4-(3'-carboxy-4'-methoxyphenylamino)-6-(4'-methoxyphenylamino)-metanilic acid.



11. 4-(4'-sulfophenylamino)-6-(4'-methoxyphenylamino)-metanilic acid.



5

12. 2,4 - bis - (phenylamino) - 5 - aminobenzoic acid.



6

19. 2,4 - di - (4' - methoxy phenylamino) - 5 - aminobenzoic acid.



13. 4 - (4' - methoxyphenylamino) - 6 - (N - carboxymethyl - N - phenylamino) - metanilic acid.



14. 4 - (4' - sulfophenylamino) - 6 - (N - carboxymethyl - N - 4' - methoxyphenylamino) - metanilic acid.



15. 4 - (2' - pyridylamino) - 6 - (N - carboxymethyl - N - 4' - methoxy-phenyl-amino) - metanilic acid.



16. 4 - (4' - methoxyphenylamino) - 6 - di - methylaminometanilic acid.



17. 4 - (4' - sulfophenylamino) - 6 - di - methylaminometanilic acid.



18. 4 - (4' - methoxyphenylamino) - 6 - (4' - methylphenylamino) - metanilic acid.



5

10

15

20

25

30

45

50

65

70

75

6



20. 2,4 - di - (phenylamino) - 5 - aminotoluene- $\omega$ -sulfonic acid.



21. 4,6-di-(methylamino)-metanilic acid.



40 22. 4 - phenylamino - 6 - methylamino - metanilic acid.



The color former which is utilized for the formation of the yellow dye image upon development is any open chain keto methylene compound, i. e., any compound containing in a straight chain a methylene group which is activated by one or more keto groups or by a keto group and a cyano or  $-\text{SO}_2$  group.

Examples of such compounds are:

1. Acetoacetanilide.
2. N-1-naphthylacetooacetamide.
3. N-1-naphthyl- $\alpha$ -benzoylacetamide.
4. N,N'-ethylenebisacetooacetamide



5. N,N'-ethylenebis- $\alpha$ -benzoylacetamide.  
6. p,p'-Bi-o-acetoacetanilide



75

7. N-2-naphthylbenzoylacetamide.

8. p,p'-Biacetooctanilide.

9. p,p'-Bi- $\alpha$ -benzoylacetanilide.10.  $\alpha,\alpha'$ -Terephthaloylbis-(3-chloro-4,6-dimethoxy-acetanilide).

22. 2-p-benzoylacetamido-benzamido-6-stearoylamino-p-toluene-sulfonic acid.

11.  $\alpha,\alpha'$ -Terephthaloylbis-(4-chloro-5-methyl-o-acetaniside).12.  $\alpha$ -Benzoylacetanilide.

13. 2-(m-benzoylacetamidophenyl)-1-octadecyl-5-benzimidazole-sulfonic acid.



14. o-Acetoacetanilide.

15. 4,4'-methylenebis- $\alpha$ -benzoylacetanilide.

16. o-Phenylacetoacetanilide.

17. 4'-2-pyridylsulfamyl- $\alpha$ -benzoylacetanilide.

18. 5,5'-ureylenebis-N-benzoylacetyl-anthra-nilic acid.



19. 3,3'-ureylenebis-6-p-benzoylacetamido-benzamido-benzene sulfonic acid.



20. p-Benzoylacetamido-benzoic acid.



21. 7-benzoylacetamido-1-naphthoxyacetic acid.



22. 2-p-benzoylacetamido-benzamido-6-stearoylamino-p-toluene-sulfonic acid.

23.  $\alpha,\alpha'$ -Terephthaloylbisacetanilide.

24. 4,4'-methylenebisacetoacetanilide.



25. p-Sulfamylbenzoylacetanilide.



26. N,N'-1-methylethylenebisaceto-acetamide



27. 2,4-pentanedione



28. 1,3-diphenyl-1,3-propanedione.

29. Benzoylacetonitrile.

30. Cyanoacetanilide.

31.  $\alpha$ -Phenylsulfonylacetophenone.

32. 2-(p-benzoylacetamidophenyl)-1-octadecyl-5-benzimidazole-sulfonic acid.

33. p-Cyanoacetyl- $\beta$ -octadecenylsuccinic acid.

Many of the above keto methylene compounds are well known, and are used, for example, as couplers in azo dye chemistry. In any case the majority can be made by the interaction of the desired amine with the desired keto ester to yield the amide.

The benzimidazole compounds, i. e., Nos. 13 and 32, are new products. Such compounds are produced, taking compound 32, for example, by

heating a mixture of 2-(4'-aminophenyl)-1-octadecylbenzimidazole-5-sulfonic acid, benzoyl acetic ester, and pyridine to a temperature of 110 to 120° C. for about four hours. The reaction mixture is then diluted with water and drowned in a mixture of concentrated hydrochloric acid and ice water. The product is collected on a filter, washed and air dried.

It may be purified by dissolving it in methanol, refluxing the solution for one-half hour, cooling to room temperature, and filtering.

Compound 13 is made in the same manner excepting that 2-(4'-aminophenyl)-1-octadecylbenzimidazole-5-sulfonic acid is replaced by 2-(3'-aminophenyl)-1-octadecylbenzimidazole-5-sulfonic acid.

The parent benzimidazole, on the other hand, is prepared by heating a 3-amino-4-alkylamino benzene sulfonic or carboxylic acid with the desired nitro benzene carboxylic acid chloride in the presence of pyridine or any other suitable acid binding agent. The nitro group in the benzimidazole is then reduced to an amino group. Preparation of the intermediate is analogous to the method described in copending application Serial No. 745,113, filed April 30, 1947, with the exception that the 1-hydroxy-2-naphthoyl chloride is replaced by the desired nitro-benzoyl chloride followed by reduction of the nitro group after ring closure. 20 25 30

In the processing of color film by the color forming development method, the general practice is to bleach the silver images after color development with a bleaching bath having a pH slightly on the acid side. Furthermore, inasmuch as it has been recognized that the cyan and magenta azine dyes are acid-resistant, it has been proposed in the method employed for forming images of such dyes to fix the silver halide after bleaching by means of an acid hardening fixing bath. This procedure has the advantage that it permits hardening of the emulsion during normal processing and without the utilization of a separate step for this purpose.

It has been the observation of operators that the processing of color film as described above, while utilizing the aforementioned 2,4-diaminoaniline color developers, and as the color former an open chain keto methylene compound, leads to dye images which are magenta rather than yellow in color. We have now found, and this constitutes a very important part of our invention, that such a magenta image is converted into a permanent yellow image by subsequent treatment with an alkali.

The alkali treatment step leading to yellow dye image formation is conducted before final washing and drying and involves merely the subjection of the photographic element being processed to the action of an aqueous solution of a water soluble alkali, such as sodium carbonate, potassium carbonate and the like. As the pH of the photographic element increases, the yellow image appears as a result of the transformation of the previously formed magenta image.

The particular stage at which the alkali treatment is interposed may vary depending upon the nature of the fixing bath employed. Generally speaking, such alkali treatment will be a final phase of the processing operation and will usually be succeeded by the final wash and drying. This order will always prevail where the fixing bath is acidic. If, however, the fixing bath is neutral, then the alkali treatment may follow bleaching and precede fixing. In any case, the

alkali treatment will be in a final phase of processing and will be subsequent to the last processing step which utilizes an acid treating bath.

The formation of the yellow dye image by color development may be illustrated by the following equations representing the use of benzoylacetanilide as the color former and 6-phenylamino-4-methylamino-metanilic acid as the color developer. It is to be understood that these equations are theoretical, being used merely to help explain the invention, and that we do not intend to be restricted thereto.



It is of course to be understood that the above compound may exist in tautomeric form. The yellow dyes thus formed appear to be true azines. Thus they withstand treatment with acid bisulfite—whereas the yellow azomethines do not. Furthermore, they are not split by treatment with dilute solutions of strong mineral acids as happens with the yellow azomethines.

The process may be carried out by utilizing the color formers in the color forming developer or in the silver-halide emulsion. Preferably, however, the color formers are located in the emulsion and are so constituted that they do not diffuse therefrom during the photographic processing. The color formers may be rendered fast to diffusion in the emulsions by methods usually employed in the art, for example, those described in United States Patents Nos. 2,178,612, 2,179,244, 2,179,234, 2,179,238, 2,179,239, 2,179,344, 2,186,045, 2,186,719, 2,186,732, 2,186,733, 2,186,734, 2,186,849, 2,186,851, 2,186,852, 2,200,306, 2,280,722, 2,292,575, 2,303,928, and 2,307,399. However, the utilization of a long aliphatic chain to render the components non-migratory has been found to give best results. Examples of compounds containing such non-diffusing groups appear above.

70 The process may be utilized for the formation of negative color images, positive color images, or of reversed color images by following the usual reversal method, i.e., exposing, developing in black and white, re-exposing, and color developing with a 2,4-diamino-aniline.

## 11

The yellow dye images produced by the present invention have excellent light fastness and brilliance and very adequately complement the magenta and cyan dyes produced by the azine process.

The following examples serve to illustrate the invention, but it is to be understood that the invention is not limited thereto.

## Example 1

To 100 ml. of a developer solution made up as follows:

|                                                |          |
|------------------------------------------------|----------|
| 6-phenylamino-4 - methylamino - metanilic acid | 8.0      |
| Metol                                          | 1.0      |
| Sodium sulfite                                 | 60.0     |
| Potassium carbonate                            | 20.0     |
| Potassium bromide                              | 10.0     |
| Benzylamine                                    | 5.0      |
| Water to                                       | 1000 ml. |

was added a solution of 0.2 gram of  $\alpha$ -benzoylacetanilide dissolved in 4 ml. of ethyl alcohol and 1 ml. of 10% sodium hydroxide solution. A strip of positive film carrying a silver halide image was treated in this developer-color-former solution for 10 minutes at 20° C. with agitation. The strip was then washed for 5 minutes in running water at 18° C. and then "bleached" in a ferricyanide-bromide bleach until all developed silver was converted into silver bromide. The strip was then washed until free from bleach and then fixed in acid-hypo. At this point the strip carried a reddish-magenta dye image which was an exact duplicate of the original silver halide image. After the strip had been washed free of hypo it was treated in a 5% solution of sodium carbonate until the reddish-magenta image was completely converted to a brilliant yellow dye image, about 1 minute being required for the conversion. The yellow image so prepared was stable to washing and drying and showed excellent light fastness and brilliance.

## Example 2

A photographic silver halide emulsion containing as a non-diffusing color former p-cyano-acetyl- $\beta$ -octadecenyl-succinalic acid having the following constitution:



is exposed, developed in black and white, re-exposed and the residual silver halide developed for 10 minutes in a developer of the composition given in Example 1. The film after development is washed 10 minutes, bleached in ferricyanide bleach and fixed in an acid hardening hypo. The strip contained a magenta dye image in duplicate of the original latent silver halide image. After the strip was washed free of hypo, it was bathed in a 5% sodium carbonate solution for 2 minutes whereupon the magenta image was converted to a yellow dye image.

## Example 3

The procedure is the same as in Example 1 excepting that the developer is made up of equal parts of 4.6-di-(phenylamino)-metanilic acid

## 12

and 4-methylamino-6 - phenylamino - metanilic acid.

Various modifications of the invention will occur to persons skilled in this art, and we therefore do not intend to be limited in the patent granted except as necessitated by the appended claims.

We claim:

1. The process of producing yellow dye images which are resistant to splitting by strong mineral acids, which comprises developing a developable silver halide emulsion in the presence of an open chain keto methylene compound with a 2.4-diamino-aniline in which the nitrogen atoms in 2- and 4-positions have directly linked thereto a carbon atom of a radical selected from the class consisting of aliphatic and aromatic radicals, bleaching and fixing said emulsion, and adjusting the pH of the emulsion in a final phase of the processing operation by treatment with an alkali until the yellow image manifests itself when the emulsion has been previously subjected to an acidic treating bath.

2. The process of producing yellow dye images which are resistant to splitting by strong mineral acids, which comprises developing a developable silver halide emulsion in the presence of an open chain keto methylene compound with a 2.4-diamino-aniline in which the nitrogen atoms in 2- and 4-positions are directly linked to the carbon atom of a radical selected from the class consisting of aliphatic and aromatic radicals, bleaching the silver formed by such development, fixing the silver salts by an acid hardening fixing bath, and subsequently adjusting the pH of the emulsion by treatment with an alkali until the yellow image manifests itself.

3. The process as defined in claim 1 wherein the open chain keto methylene compound contains a benzoylacet radical.

4. The process as defined in claim 2 wherein the 2.4-diamino-aniline is 6-phenylamino-4-methylamino-metanilic acid and wherein the open chain keto methylene compound is  $\alpha$ -benzoylacetanilide.

5. The process as defined in claim 2 wherein the 2.4-diamino-aniline is 6-phenylamino-4-methylamino-metanilic acid and wherein the open chain keto methylene compound is p-cyano-acetyl- $\beta$ -octadecenylsuccinalic acid.

6. The process as defined in claim 2 wherein the 2.4-diamino-aniline is composed of a mixture of equal parts of 4.6-di-(phenylamino)-metanilic acid and 4-methylamino-6-phenylamino-metanilic acid and the open chain keto methylene compound is  $\alpha$ -benzoylacetanilide.

7. The process as defined in claim 1 wherein the pH is adjusted by means of a 5% solution of sodium carbonate.

8. The process as defined in claim 2 wherein the pH is adjusted by means of a 5% solution of sodium carbonate.

DONALD E. SARGENT.  
ROBERT C. GUNTHER.

## REFERENCES CITED

The following references are of record in the file of this patent:

## 70 UNITED STATES PATENTS

Number Name Date  
2,414,491 Tulagin Jan. 21, 1947